

## UNITED STATES PATENT OFFICE

PAUL EMMITT WHITE, OF LANCASTER, OHIO

## METHOD OF CASTING TYPE FACES, STEREOTYPE, ETC.

No Drawing.

Application filed December 4, 1930. Serial No. 500,134.

The invention herein described has to do primarily with the printing art, although the apparatus may be used in other arts where conditions and results would be similar, therefore I do not wish to limit the scope of this invention or its application to that branch of the printing art herein used to illustrate my invention, although the apparatus and method as herein disclosed is particularly adapted to that branch of printing embracing the casting of type or stereotype and the like.

Heretofore in the casting of stereotype from a stereotype mat great losses have occurred and much valuable time has been consumed in the casting of the stereotype plates from a mat that has been previously used or from a mat which has become warped or distorted, or from a freshly made mat.

Further, it is not uncommon for a mat to absorb moisture in varying degrees over its face or surface whereby steam or gases are evolved when the hot metal is cast thereon causing a blurring or imperfections that are troublesome and unsatisfactory.

Again, it is well known by those skilled in the art that certain type faces will produce a cleaner cut and better printing face from a stereotype mat than will others where the ordinary procedure of casting the stereotype is followed.

Further, it is difficult to obtain a clear cut casting of a picture even from the first pouring on a new mat by the usual method and substantially impossible to get a satisfactory casting from an old or used mat, whereas castings made by my improved method are more perfectly defined, clearer cut and free from smudges, cold shots and other imperfections.

These three faults are particularly annoying and at times are the cause of delays and a loss of time which is invaluable.

My method of casting fluid metals for the purpose of obtaining accurate reproduction of the mat surface and the results as also the problem in the casting of stereotype or type faces is quite different from that where the interior of the metal is required to be homogeneous, and in the invention here disclosed one is required to deal with only the exterior surface of the casting irrespective of its homo-

geneity and density and for this reason the amplitude and frequency of the vibrations transmitted to the metal during casting and during the cooling of the metal to the point of solidification are of prime importance in that by my herein disclosed method I overcome the power of surface tension and because of the continued cooling of the metal the resulting increase of viscosity which prevents the metal from flowing into minute recesses and lines, depressions or acute angles of configuration.

Because of the character of the material from which the mat or mold surface is formed, it is desirable to make castings of type metal at as low a temperature as is possible and obtain perfect type faces thereby preserving the mat and also reducing the loss of metal by oxidation and formation of dross, but when the ordinary procedure is followed it is not an infrequent occurrence that, because of the variation and character of the letters and impressions in the mat, it is necessary to raise the temperature of the metal 50° or possibly 75° above normal or the mean temperature at which the major portion of the surfaces would be cast and this usually results in decreasing the life of the mat and in some instances totally destroying the same or making it unusable to obtain further castings.

Now my invention consists of a means for rapidly vibrating the casting box or foundation that carries the mold mat and I have found that this can best be accomplished by applying one or more of the ordinary electric vibrators or modifications thereof to the casting box, as is used in vibrating sand molds or the patterns so prevalently used in foundry practice. To carry out my method I arrange one or more of these electric vibrators on a desirable part of the casting box so that when the same is put in operation it produces a vibration of the metal casting box which is transmitted to the mat. I have found in certain instances that it is desirable to use a special form of these vibrators, one that is so constructed as to permit regulating the force as also the frequency of the blow.

I deem it unnecessary to describe in detail the construction of the vibrating appa-

55

60

65

70

75

80

85

90

95

100

ratus for I can use, with varying degrees of efficiency, any of the common or well known foundry vibrators, therefore, it seems unnecessary to illustrate the manner of applying the vibrator to the casting box. I believe that I can adequately describe the method of using the vibrator and the results flowing therefrom as the apparatus is so universally used and so varied in construction 10 that a detailed illustration of construction is unnecessary.

Now referring to the defects above enumerated, the effect of my invention in overcoming them is as follows:

15 Very annoying and harmful but prevalent condition is met when the mat is warped and does not lie down in a perfect plane or in contact with the casting box frame, however, when the operator starts to pour the metal 20 into the gate he actuates a switch and starts the vibrator and these vibrations together with the weight of molten metal forces the mat into contact with the plane surface of the casting box plate thereby producing a 25 lettered surface that is sharp and uniform.

Further, vibrating the mold frame and mat agitates the metal during its progress into the recesses or corners, edges, etc., of the letters or the mold and forces out any gas or 30 air that has become entrapped or entrained in the metal.

Further, it is obvious that the fluid metal when agitated in this manner will more readily flow into corners or narrow and extended paths which will not be filled if it 35 is not agitated. Here it is well to point out that, contrary to the belief and suggestions of some, this method of casting gives results very different from those obtained by casting under pressure of vacuum for the reason that the agitation of the metal not only creates heat but it also shifts substantially instantly any portion of metal which has become sufficiently cooled as to be partially 40 congealed or whose viscosity has increased to a point where pressure would not move it. Also, vibration produces a constant distortion of any portion of fluid metal which would be subject to such a condition that 45 the effect of vibration substantially prevents the configuration of any congealed portion or the effect of cooling upon the character of the impressions obtained.

The fact that first class or perfect impressions can be obtained at lower temperatures by vibrating the metal has a decided advantage, both as to the quality of the finished work as also the cost, because the lower the temperature at which the metal is cast the 50 better, for if the temperature of the metal is increased above 525° F., deterioration is greatly increased and oxidized or "burnt" metal is often the cause of imperfect castings, particularly half-tones or pictures and 55 shadings.

My invention and its use involves no large expense, maintenance or operating costs nor increased labor, for the amount of current required to operate the vibrator and the original cost, considering the operative life of the 70 equipment, are very small.

Having described my invention I claim the following:

1. A method of making printing plates which consists in placing a mat in a mold box, holding the mat in position therein, pouring molten metal into the mold box and vibrating the mold box and the metal during the period of pouring whereby any warpage 75 of the mat is overcome and a perfect impression obtained.

2. A method of removing gases entrapped between a mat and molten metal poured thereon to form a stereotype casting, which includes the steps of placing the mat in a mold box, pouring molten metal on the mat, and vibrating the metal and the mat whereby the fluid metal displaces gases remaining in recesses or pores in the surface of the mat. 85

3. A method of making stereotype castings including the steps of placing a mat in a mold box, holding the mat in a stationary position therein, casting fluid metal in the mold, vibrating the mold and the metal, and regulating the amplitude and frequency of the vibrations during the casting process to cause the vibrating metal to press the mat firmly against the mold regardless of any warpage in the mat. 90

4. A method of casting a printing plate 100 including the steps of pouring molten metal into a mold having a mat therein, and vibrating the mold while the metal therein is still plastic to force the metal into the crevices of the mat against the effect of the surface of the mat, the surface tension of the molten metal and its viscosity. 105

5. A method of casting a printing element including placing a mat in a mold, pouring molten metal on the mat, vibrating the mold 110 while said metal is still plastic, to force the metal into the crevices of said mat against the effect of the surface of the mat, and the surface tension and viscosity of the metal in opposing flow of the metal, and continuing the vibration until the metal is substantially set. 115

In testimony whereof I have hereunto set my hand, this 26th day of November, 1930, at Lancaster, Ohio.

PAUL E. WHITE.

125

130